

(No Model.)

P. & C. P. APPEL & C. W. HIRRLINGER.  
Incrusting and Enameling Precious Stones.

No. 240,496.

Patented April 26, 1881.

Fig: 1.



Fig: 2.



WITNESSES:

Carl Karp.  
Richard Fischmann.

INVENTOR

Peter Appel, Charles P. Appel, and  
Charles W. Hirrlinger.

BY

Peter Appel,  
ATTORNEY.

# UNITED STATES PATENT OFFICE.

PETER APPEL AND CHARLES P. APPEL, OF WEST HOBOKEN, NEW JERSEY,  
AND CHARLES W. HIRRLINGER, OF NEW YORK, N. Y.

## INCRUSTING AND ENAMELING PRECIOUS STONES.

SPECIFICATION forming part of Letters Patent No. 240,496, dated April 26, 1881.

Application filed May 13, 1880. (No model.)

*To all whom it may concern:*

Be it known that we, PETER APPEL and CHARLES P. APPEL, of West Hoboken, in the county of Hudson and State of New Jersey, and CHARLES W. HIRRLINGER, of New York, in the county and State of New York, have invented certain new and useful Improvements in Incrusting and Enameling Precious Stones, of which the following is a specification.

10 This invention relates to an improved method of incrusting and enameling precious stones, such as onyx and agate; and it consists in first engraving the design into the stone to be ornamented, then pressing or molding a thin 15 plate of gold into the indentation, then removing, enameling, and burning the plate, next replacing and cementing the plate into the stone and finally grinding the surface of the 20 enameled portions flush with the surface of the stone.

In the accompanying drawings, Figure 1 represents a side elevation; and Fig. 2, a detail 25 vertical transverse section of a ring, on line  $x$ - $x$ , Fig. 1, which is incrusted and enameled according to our improved method.

Similar letters of reference indicate corresponding parts.

A in the drawings represents a round, flat, or other shaped piece of onyx, agate, or other 30 precious stone to be ornamented. This stone is preferably set onto a frame, B, of gold or other metal, in such a manner that the side flanges of the frame are flush with the surface of the stone, so as to protect the same against 35 breakage. The surface of the stone is ornamented with incrusted gold of different colors, and with enameled portions, in the following manner:

The design to be produced is first engraved 40 into the stone, the portions to be enameled being cut of greater depth than the portions which are to be incrusted merely. Into the deeper portions or indentations thin plates C, of gold or other metal, are pressed until they assume 45 the exact shape of the indentations, the plates being then trimmed so as to correspond exactly to the outlines of the portion to be en-

ameled. The plates C are next removed from the recess and enameled in the usual well-known manner. After the colors are burned 50 into the enamel in a muffle the gold plates are replaced and cemented into the indentations, and finally ground off, so as to be flush with the surface of the stone and surrounding casting.

55 The novel feature of our method, to which we specially draw attention, is that the enameled and incrusted portions are entirely embedded into and flush with the surface of the stone, giving it a highly-ornamental appearance, as the enamel is surrounded by a narrow band of gold. The enameled portions, being flush with the surface, are not liable to wear off, as the enamel is when laid on the surface of the stone, so that the articles of jewelry retain 65 always their finished original appearance.

Having thus described our invention, we claim as new and desire to secure by Letters Patent—

1. The method herein described of incrusting and enameling precious stones, consisting in engraving the design upon the stone, then molding a thin plate in the engraved portions, then removing and enameling the plate, next cementing it into the recess, and finally grinding the surface of the enameled plate flush with the surface of the stone, substantially as set forth.

70 75 2. As a new article of manufacture, a precious stone for jewelry having incrusted and enameled ornaments set into recesses flush with the surface of the stone, substantially as specified.

In testimony that we claim the foregoing as our invention we have signed our names, in 80 presence of two witnesses, this 12th day of May, 1880.

PETER APPEL.  
CHAS. P. APPEL.  
CHARLES W. HIRRLINGER.

Witnesses:

PAUL GOEPEL,  
CARL KARP.